

Oct. 16, 1951

J. G. BOS ET AL

2,571,670

METHOD OF PRODUCING PHOTOGRAPHIC CONTRASTS

Filed Jan. 21, 1947

2 SHEETS—SHEET 1



Fig. 1.



Fig. 2.



Fig. 3. INVENTORS  
JULIUS GOEMAN BOS, CORNELIS JOHANNES DIPPEL  
HARKE JAN HOUTMAN, KLAAS JANNES KEUNING & SJOERD  
BY WINTZES *W. M. Vogel*  
AGENT

Oct. 16, 1951

J. G. BOS ET AL  
METHOD OF PRODUCING PHOTOGRAPHIC CONTRASTS

2,571,670

Filed Jan. 21, 1947

2 SHEETS—SHEET 2



INVENTORS  
JULIUS GOEMAN BOS,  
CORNELIS JOHANNES DIPPEL,  
HARKE JAN HOUTMAN,  
KLAAS JANNES KEUNING,  
& SUOERD WINTZES

BY *Jan M. Vogel*

AGENT

## UNITED STATES PATENT OFFICE

2,571,670

## METHOD OF PRODUCING PHOTOGRAPHIC CONTRASTS

Julius Goeman Bos, Cornelis Johannes Dippel,  
 Harke Jan Houtman, Klaas Jannes Keuning,  
 and Sjoerd Wijtzes, Eindhoven, Netherlands,  
 assignors to Hartford National Bank and Trust  
 Company, Hartford, Conn., as trustee

Application January 21, 1947, Serial No. 723,426  
 In the Netherlands January 21, 1946

4 Claims. (Cl. 95—5)

1

This invention relates to a method of producing photographic contrasts, more particularly to material sensitized by means of a diazonium compound, and is of particular importance for the manufacture of copies of image and sound films, since it permits contrasts having different gamma values to be obtained side by side on one and the same material.

It is known that photographic material sensitized by means of light-sensitive diazonium compounds often exhibit contrasts, the graduation of which is unsatisfactory. Thus, for example, physically developed metal images obtained by using diazonium compounds and metal compounds, e. g. a mercurous salt, reducible in an aqueous medium often have a gamma value of from 6 to 7. This is to be understood to mean the maximum value of the gamma i. e. the maximum value of the gradient of the characteristic blackening curve. Such a gamma value is very suitable for making copies of sound records by means of width variations and particularly for copying a mechanically produced sound track (cf. French patent specification 817,850). However, for copying, for example, image negatives and sound records by means of depth variations it is much too high.

It has now been found that with the aforesaid material the gamma value may depend upon the moisture content of the material at the moment of exposure. In a copending United States patent application Serial No. 727,310 filed February 8, 1947, exclusive rights have been claimed for a method of controlling the gradation of a photographic contrast, in which this phenomenon is utilized. It has, however, further been found that with this kind of material the gamma value of the contrast may also vary according as the intensity and duration of the exposure vary, notably if the material has an increased moisture content.

According to the present invention, the gradation of a material having a gamma value dependent upon the moisture content is controlled by varying the intensity and duration of the exposure, particularly with an increased moisture content of the material. The intensity of exposure is to be understood to mean the flux per  $\text{cm}^2$  of the photo-chemically active light falling on the sensitized material. On varying the intensity and duration, that intensity and duration should be compared which, under the conditions used in regard to blackening and so on, yield the same blackening, for instance a blackening exceeding the fog by 0.05.

5 A material having a gamma value dependent upon the moisture content is to be understood to mean a material with which a variation of the moisture content, under otherwise the same conditions, is capable of bringing about at least a variation of the ratio 1:1.2 in the gradient of that part of the characteristic blackening curve having blackenings of from 0.4 to 1.5. For comparison tests this gradient should naturally be measured at the same blackenings. The material is considered to have an increased moisture content if the moisture content of the part of the material being photo-chemically active in the production of contrasts at least exceeds the moisture content which this part would have if the material should be in equilibrium with an atmosphere having a relative degree of moisture of 65% at 20° C.

10 It is pointed out that apart from and in addition to the method of gamma control according to the invention other methods of influencing the gamma remain serviceable. This is obvious, for external methods such as the arrangement of a grating closely in front of the photographic material (cf. French patent specification 848,531); this applies, however, also to methods in which use is made of a so-called internal grating (cf. French patent specification 841,911), of a variation 15 of the composition of developing and sensitizing liquid, of a variation in developing time, of a variation in wavelength of the exposure. The method according to the invention permits of being very effectively combined with the aforesaid method consisting in varying the moisture content of the material at the moment of exposure. By combining the method according to the invention with one of the last-mentioned methods, ample variation of the gamma value is often obtainable whilst retaining a sufficient maximum blackening and avoiding a grating structure.

20 The use of the invention permits of obtaining excellent results in producing photographic contrasts, particularly metal images, by means of photographic material sensitized by a light-sensitive diazonium compound.

25 This applies particularly to the production of photographic, physically developed metal contrasts by means of a sensitized oxydiazonium compound and a mercurous salt. Contrasts thus obtained are grainless, i. e. the grains are smaller than  $1\mu$ . If a film made from regenerated cellulose and impregnated with a light-sensitive oxydiazonium compound and a mercurous salt, 30 is exposed at high intensity in a moist state and

35 40 45 50 55

then physically developed to a neutral grey tone, a maximum gamma value of at least 4 is readily obtained. By exposing the same material at a low intensity, a gamma value of from 1.5 to 2 is obtainable, whilst retaining a sufficient maximum blackening and a neutral grey tone. This renders the material very suitable, for example, for the manufacture of image positives suitable for projection.

A very important advantage of the invention consists in that it permits of producing side by side, on one and the same material, contrasts having different gradations, by effecting the exposure required for obtaining the various graduated contrasts, with different intensity and duration, particularly at an increased moisture content of the sensitized material. Owing to this, it is of much importance for the manufacture of sound film copies with which one and the same film band is provided with images and sound records and with which different gradations for image and sound are desired. Photographic material of the aforesaid kind, which consists of a transparent support, for example regenerated cellulose treated with a sensitized diazonium compound and a mercurous salt, and is physically developed after the exposure, permits of manufacturing, for example, soundfilm copies having an image of low gamma value and a sound record of high gamma value. For this purpose the image band and the sound record are copied at a different exposure intensity and duration. The development of the exposed copy is preferably effected in one operation; in spite thereof, different gradations are obtained for the image part and the sound part of the copy. Copies thus obtained are cheap and of excellent quality.

In this embodiment, in which a film is provided with contrasts located side by side and having different gradations, the film is preferably passed in one continuous operation in front of the exposure apparatus for copying image and sound the desired exposure time being determined by a judicious choice of the distance the moving film is exposed to the action of the copying light and the desired intensity being obtained, for example, by a suitable choice of the intensity and distance of the source of light.

Furthermore, the invention, on copying a pictorial film, permits of obtaining different gradations for succeeding series of images. For example, in the case of a succession of scenes, the gradation desired for each scene may be obtained by providing for suitable exposure conditions on copying. This is of particular importance for the manufacture of copies of film reports, such as film news-reels. If desired, the exposure conditions may automatically be adjusted to the best values by providing the film strip to be copied with a control track which controls, for example by photoelectric means, the intensity and duration of the exposure.

Another use of the possibility to provide different gradations on one and the same material consists in that different parts of a single image are given different gradations. On copying a portrait or a landscape, for example, the background and the air respectively may be given different gradations. This use may be of importance for enlargement or for the transmission of photographic images by television or the like.

The relation existing between the exposure conditions and the gamma value obtained depends upon various factors, such as the nature of the support, the quantity of the light-sensitive com-

ound in the support and so forth, but can be determined experimentally.

A very important factor is the moisture content of the support. As stated things are even such that in the case of a constant exposure intensity a variation of the moisture content permits the gamma to be controlled. Consequently, for the obtainment of reproducible results, a reproducible adjustment of the moisture content is of much importance. A very reliable control of the moisture content is ensured by bringing the material in equilibrium with an atmosphere of suitable relative humidity, which may be effected by leaving the material for a sufficiently long time, a film band of regenerated cellulose for example for 24 hours, in such an atmosphere.

It is, however, not necessary that the material should be in a state of equilibrium with respect to moisture content. It is sufficient that the moisture content has the value required in regard to the desired gradation in the zone of the material where the photo-chemical conversion takes place. This permits a much quicker adjustment of the moisture content than in the case of waiting for the state of equilibrium. If, for example, an increased moisture content is desired, the moisture content of the photo-chemically active part of the material is adapted to be adjusted to the desired value in a very short time by treating the sensitized material with water and by drying it slightly or conversely by introducing dry material into a moist atmosphere. It is to be noted that the moisture content of the material at the moment of exposure is vital. It has been found that in this manner a reliable and reproducible control of the gamma value is readily possible. The gamma value obtained does not depend upon variations of the moisture content after exposure.

On adjusting the moisture content, apart from the method by means of which this is carried out, the nature of the material should be considered. For example, if a light-sensitive diazonium compound is introduced into gelatine, the material must be in equilibrium with an atmosphere having a different humidity in order to obtain the same moisture content as with regenerated cellulose.

To obtain good results, it is, naturally necessary that the material which contains the light-sensitive compound is capable of absorbing moisture. Excellent results are obtained by means of regenerated cellulose. The support as a whole is not required to be capable of absorbing moisture, it being sufficient that the part of the support containing the photo-chemically active compound is capable of absorbing water. Very suitable is, for example, a superficially saponified cellulose acetate or a support sensitive or not sensitive to moisture which carries a water-absorbing layer, for example, gelatine or another albumin or albuminous product containing the light sensitive compound. As an alternative, use may be made of a material entirely or partly consisting of polycondensation products, such as polyamides.

The invention will be explained more fully with reference to the accompanying drawings, which represent characteristic curves obtained under different conditions of exposure and with different moisture contents. The curves are inferred from the blackening variation of contrasts obtained under a sensitometer wedge.

#### EXAMPLE

ing it in a solution of 0.1 n hydroxy-1 diazonium-2 methyl-6 benzene sulphonic acid-4, 0.025 n mercurio-nitrate and 0.05 n nitric acid followed by conditioning at 22° C. and a relative humidity of 40, 75, 90 and 96% respectively by leaving the material for a considerable time in an atmosphere having such a degree of humidity and temperature.

After that it was exposed by means of a Philips superhigh-pressure mercury-vapour lamp of 500 watts under a sensitometer wedge. After the exposure the material was washed in distilled water, developed at 22° C. in a solution of 2% metol (sulphate salt of p-methyl-aminophenol), 4% tartaric acid and 0.4% silver nitrate, the time of development being 3 minutes for the material conditioned to 40% and 2 minutes for the remainder.

The characteristic curves were derived from the contrasts obtained, whereupon the gradations of the contrasts could be determined. The gradations obtained under different conditions of exposure are stated in the table.

The first and second column indicate the time of exposure and the distance of the exposure lamp from the sensitized material, the following columns stating, under the headings 40, 75, 90 and 96% R. H. (the relative humidities R. H. at which the conditioning took place), the numbers of the gamma value of the contrasts obtained. The table states the gradient of the characteristic curve at a blackening 1.

If the distance of the exposure lamp should have a value different from that indicated in the second column, this deviating value is stated between brackets behind the gradient found.

Figs. 1 to 4 show the characteristic blackening curves as found under conditioning circumstances of 40, 75, 90 and 96% of relative humidity respectively. The values stated at the abscissa refer to relative values of  $\log I$ .

Table

| time of exposure in seconds | lamp distance in cm. | 40% R. H.  | 75% R. H. | 90% R. H.  | 96% R. H.  |
|-----------------------------|----------------------|------------|-----------|------------|------------|
| 0.46                        | 4.0                  | 7.0 (3.2)  | 9.0       | 8.5        | 2.6        |
| 1.5                         | 6.0                  | 6.3 (5.2)  | 7.4       | 7.6        | 1.9        |
| 4.6                         | 9.0                  | 6.2        | 6.5       | 4.6        | 1.2 (10.8) |
| 10.7                        | 19.5                 | 6.0 (16.2) | 5.6       | 3.0        |            |
| 30.0                        | 28.1                 | 5.3        | 3.2       | 2.3 (32.5) |            |
| 90                          | 48.5                 | 4.8        | 2.8       |            |            |
| 270                         | 59                   | 4.0        |           |            |            |
| 980                         | 94                   | 3.8        |           |            |            |

What we claim is:

1. In the process of producing photographic contrasts on a transparent cellulosic moisture absorbent carrier having a given initial moisture content and supporting a light-sensitive system containing a diazonium compound and a reducible mercurous salt, the steps comprising varying the moisture content of one portion of said carrier to an extent at which the resultant moisture content of said portion has a value which corresponds to a state of equilibrium between said portion and an atmosphere having a relative humidity of about 40 to 96%, varying the moisture content of a second portion of the carrier to an extent at which the resultant moisture content of said second portion has a value different than the moisture content of said first portion and has a value which corresponds to a state of equilibrium between said second portion and an atmosphere having a relative humid-

ity of about 40 to 96%, exposing the first portion containing the said moisture content to the action of light having a given intensity of illumination to form a photographic contrast thereon having a given gamma value, and exposing the second portion containing the said moisture content to the action of light having an intensity different from said given intensity to form a photographic contrast thereon having a gamma value different from said given gamma value.

2. In the process of producing photographic contrasts on a carrier comprising a transparent cellulosic and a moisture absorbent albuminous base thereover, said carrier having a given initial moisture content and supporting a light-sensitive system containing a diazonium compound and a reducible mercurous salt, the steps comprising varying the moisture content of one portion of said carrier to an extent at which the resultant moisture content of said portion has a value which corresponds to a state of equilibrium between said portion and an atmosphere having a relative humidity of about 40 to 96%, varying the moisture content of a second portion of the carrier to an extent at which the resultant moisture content of said second portion has a value different than the moisture content of said first portion and has a value which corresponds to a state of equilibrium between said second portion and an atmosphere having a relative humidity of about 40 to 96%, exposing the first portion containing the said moisture content to the action of light having a given intensity of illumination to form a photographic contrast thereon having a given gamma value, and exposing the second portion containing the said moisture content to the action of light having an intensity different from said given intensity to form a photographic contrast thereon having a gamma value different from said given gamma value.

3. In the process of producing photographic contrasts on a transparent cellulosic moisture absorbent carrier having a given initial moisture content and supporting a light-sensitive system containing a diazonium compound and a reducible mercurous salt, the steps comprising varying the moisture content of a picture record portion of said carrier to an extent at which the resultant moisture content of said portion has a value which corresponds to a state of equilibrium between said portion and an atmosphere having a relative humidity of about 40 to 96%, varying the moisture content of a sound record portion of the carrier to an extent at which the resultant moisture content of said sound record portion has a value different than the moisture content of said first portion and has a value which corresponds to a state of equilibrium between said second portion and an atmosphere having a relative humidity of about 40 to 96%,

exposing the picture record portion containing the said moisture content to the action of light having a given intensity of illumination to form a photographic contrast thereon having a given gamma value, and exposing the sound record portion containing the said moisture content to the action of light having an intensity different from said given intensity to form a photographic contrast thereon having a gamma value different from said given gamma value.

4. In the process of producing photographic contrasts on a superficially saponified cellulose carrier having a given initial moisture content and supporting a light-sensitive system containing a diazonium compound and a reducible mercurous salt, the steps comprising varying the moisture content of one portion of said carrier to an extent at which the resultant moisture content of said portion has a value which corresponds to a state of equilibrium between said portion and an atmosphere having a relative humidity of about 40 to 96%, varying the moisture content of a second portion of the carrier to an extent at which the resultant moisture content of said second portion has a value different than the moisture content of said first portion and has a value which corresponds to a state of equilibrium between said second portion and an atmosphere having a relative humidity of about 40 to 96%, exposing the first portion containing the said moisture content to the action of light having a given intensity of illumination to form a photographic contrast thereon having a given gamma value, and exposing the second portion containing the said moisture content to the action of light having an intensity different from said given intensity to form a photo-

graphic contrast thereon having a gamma value different from said given gamma value.

5 JULIUS GOEMAN BOS.  
CORNELIS JOHANNES DIPPEL.  
HARKE JAN HOUTMAN.  
KLAAS JANNES KEUNING.  
SJOERD WIJTZES.

## REFERENCES CITED

10 The following references are of record in the file of this patent:

## UNITED STATES PATENTS

| Number       | Name           | Date           |
|--------------|----------------|----------------|
| 15 466,534   | Charlton       | Jan. 5, 1892   |
| 1,396,770    | Mees           | Nov. 15, 1921  |
| 1,710,455    | Langguth       | Apr. 23, 1929  |
| 1,861,918    | Hickman        | June 7, 1932   |
| 1,966,755    | D'Hauterive    | July 17, 1934  |
| 20 1,997,507 | Akintievsy     | Apr. 9, 1936   |
| 2,067,690    | Alink          | Jan. 12, 1937  |
| 2,106,868    | De Boer        | Feb. 1, 1938   |
| 2,183,447    | Dippel         | Dec. 12, 1939  |
| 2,196,110    | Eggers         | Apr. 2, 1940   |
| 25 2,252,006 | Holst          | Aug. 12, 1941  |
| 2,256,356    | Russell et al. | Sept. 16, 1941 |
| 2,269,161    | Morse          | Jan. 6, 1942   |

## FOREIGN PATENTS

| Number     | Country       | Date          |
|------------|---------------|---------------|
| 30 480,352 | Germany       | Aug. 8, 1929  |
| 377,145    | Great Britain | July 21, 1932 |
| 735,718    | France        | Sept. 6, 1932 |
| 853,868    | France        | Dec. 16, 1939 |

## OTHER REFERENCES

35 Eder, "The Inland Printer," Oct. 1925, pp. 91-93.